

## UNITED STATES PATENT OFFICE

2,155,410

## PRODUCTION AND TREATMENT OF ARTIFICIAL TEXTILE MATERIALS CONTAINING ORGANIC DERIVATIVES OF CELLULOSE

Henry Dreyfus, London, England

No Drawing. Application February 4, 1936, Serial No. 62,329. In Great Britain March 7, 1935

7 Claims. (Cl. 18—54)

This invention relates to improvements in the production and treatment of artificial materials, and particularly to improvements in processes wherein artificial filaments, yarns and similar textile materials containing organic derivatives of cellulose are stretched.

It is known that by stretching artificial filaments and similar materials having a basis of organic derivatives of cellulose their physical properties, and particularly their tensile strength, may be improved. It is possible, however, to stretch artificial filaments, yarns and similar textile materials by only a relatively small extent, for example about 20 to 25%, when they are in a finished condition, and in order that a higher degree of stretching may be achieved, it is in general necessary to bring the materials to a softened condition, for example by treatment with volatile solvents.

It has now been discovered that when artificial filaments, yarns and similar textile materials of organic derivatives of cellulose contain plasticisers of high compatibility they can be stretched to an exceptional extent without the necessity for treating them with softening media, and according to the present invention, therefore, artificial filaments, yarns and similar textile materials having a basis of organic derivatives of cellulose and containing plasticisers for such cellulose derivatives which are compatible therewith in high proportions, are subjected to a stretching operation.

The invention is of particular importance in connection with the manufacture of artificial filaments, yarns and similar textile materials having a basis of cellulose acetate, but it is also applicable generally to the manufacture of artificial textile materials having a basis of other organic derivatives of cellulose, for example cellulose formate, cellulose propionate, cellulose butyrate, cellulose nitro-acetate and other cellulose esters and mixed esters, methyl cellulose, ethyl cellulose, butyl cellulose and other cellulose ethers and mixed ethers, and cellulose ether-esters, e. g. ethyl cellulose acetate and oxyethyl cellulose acetate.

As stated above the plasticisers employed according to the present invention are compatible with the cellulose derivatives in high proportions, e. g. 50—70% or more. It is preferable that the plasticisers should be compatible in proportions of 100% or more on the weight of the cellulose derivative. Suitable plasticisers are tartrate esters, e. g. dibutyl tartrate and diethyl tartrate, phthalate esters, e. g. dimethyl phthalate, diethyl phthalate, dimethyl glycol phthalate, diethyl glycol phthalate, and dibutyl glycol phthalate, triethyl citrate, cresyl glyceryl diacetate, methyl cyclohexanyl oxalate, benzyl benzoate, triacetin, triphenyl-acetin, aromatic sulphonamides and

alkyl substitution derivatives thereof, e. g. para-toluene sulphonamide and the isomeric xylene sulphonamides, and benzyl alcohol.

The plasticisers may be incorporated in the artificial textile materials by introducing them into the spinning solutions and forming the solutions into the artificial textile materials by dry spinning processes. Wet spinning processes may also, if desired, be employed. When textile materials are formed by wet spinning processes from solutions containing plasticisers, the coagulating conditions should be such that a substantial proportion of plasticiser remains in the materials after they have been withdrawn from the coagulating bath.

The plasticisers are preferably present in the materials to be stretched in substantial proportions, e. g. in proportions of 40—60% up to 80—100% or more, based on the weight of the cellulose derivative.

Artificial filaments, yarns and similar textile materials may be stretched in the form of hanks or other packages, but preferably stretching is effected during the course of their travel from one point to another, for example during their transfer from one bobbin to another. It is of particular advantage to stretch a plurality of yarns simultaneously whilst they are spaced apart in parallel alignment and substantially in sheet formation, by means of devices stretching across the entire sheet. Again, artificial filaments and like materials may be stretched during their travel from spinning machines in which they have been produced to suitable winding devices. The stretching may be effected in a single stage or in two or more stages with or without intermediate stages during which the materials are released from the stretching tension.

Stretching of the materials may be effected at normal temperatures, particularly if they contain high proportions of plasticisers. Preferably, however, particularly if high degrees of stretch are to be effected, e. g. stretches of 200%, 400% or more of the original length of the materials, the stretching operation is carried out at increased temperatures, for example by passing the materials through a vessel containing a suitable gas or vapour, e. g. wet or dry steam or air under normal or superatmospheric pressure, or a suitable liquid, e. g. hot water, such gas, vapour or liquid being maintained at a suitable temperature, e. g. 50 to 100° C. or 120° C. or above. Artificial filaments and the like may be stretched to a comparatively small extent, e. g. to 150 or 200% of their original length, or, if desired, considerably higher stretches may be effected, for example to 400 or 600% or more of their original length.

The plasticisers or a proportion thereof may be removed from the filaments or other textile ma-

15

20

25

30

35

40

45

50

55

60

terials during or after the stretching operation. Thus the stretching may be effected at high temperatures by passing the textile materials containing the plasticisers through hot liquids which are solvents for the plasticiser and thus remove it from the materials during the stretching operation. The plasticisers may be wholly or partly removed from the materials after the stretching operation by any suitable method, e. g. by treating the materials with a liquid which is a solvent for the plasticiser employed and is a non-solvent for the organic derivatives of cellulose. Examples of suitable liquids are hydrocarbons and chlorinated hydrocarbons, e. g. benzene, toluene, dichlorethylene, and carbon tetrachloride, ethers, e. g. diethyl ether and di-isopropyl ether, and alcohols, e. g. methyl alcohol and ethyl alcohol. Water or aqueous solutions of suitable liquids, e. g. aqueous solutions of alcohols, may also be employed.

The following examples illustrate the invention but are not to be regarded as limiting it in any way:—

*Example 1*

25 Yarns of cellulose acetate containing dibutyl tartrate in a proportion of about 70% of the weight of the cellulose acetate are led from a creel of bobbins and passed through a reed in warp formation. Whilst in this formation the yarns 30 are led through a vessel containing air at a temperature of 150°-200° C. or water at a temperature of 90°-100° C. and are simultaneously stretched. Dibutyl tartrate remaining in the materials after the stretching operation is removed 35 therefrom by treatment with hydrocarbon solvents.

*Example 2*

40 Filaments of cellulose acetate are formed by dry spinning a solution of cellulose acetate containing 60-70% on the weight of the cellulose acetate of para-toluene sulphonamide. Such filaments, during their travel from the spinning 45 chamber to a winding device, are passed through a chamber containing wet steam at superatmospheric pressure, and are simultaneously stretched. The plasticizer in the materials is subsequently removed, at least in part, by treatment of the materials with ethyl alcohol.

50 Having described my invention what I desire to secure by Letters Patent is:

1. Process for the manufacture of artificial textile materials of improved properties, which comprises stretching at temperatures of at least 50° C. artificial filaments, yarns and like textile materials having a basis of an organic derivative of cellulose, containing a proportion of at least 40% on the weight of the cellulose derivative of a plasticizer for such cellulose derivative which is compatible therewith in a proportion of at least 50% and containing substantially no volatile softening agent.

65 2. Process for the manufacture of artificial textile materials of improved properties, which comprises forming artificial filaments, yarns and like textile materials having a basis of an organic derivative of cellulose and containing at least 40% of their weight of a plasticizer for the organic derivative of cellulose which is compatible therewith in a proportion of at least 70% by an evaporative process from a spinning solution con-

taining the organic derivative of cellulose and the plasticizer, and then stretching the materials at a temperature of at least 50° C. to at least 150% of their original length during their travel from one point to another while they are substantially free from volatile softening agent. 5

3. Process for the manufacture of artificial textile materials of improved properties, which comprises stretching at temperatures of at least 50° C. during their travel from one point to another artificial filaments, yarns and like textile materials having a basis of an organic derivative of cellulose, containing a proportion of at least 40% on the weight of the cellulose derivative of a plasticizer for such cellulose derivative which is compatible therewith in a proportion of at least 70% of the weight of the cellulose derivative and containing substantially no volatile softening agent.

4. Process for the manufacture of artificial 20 textile materials of improved properties, which comprises stretching to at least 150% of their original length and during their travel from one point to another at temperatures of at least 50° C. artificial filaments, yarns and like textile 25 materials having a basis of cellulose acetate, containing a proportion of at least 60% on the weight of the cellulose acetate of a plasticizer for the cellulose acetate which is compatible therewith in a proportion of at least 70% and containing 30 substantially no volatile softening agent.

5. Process for the manufacture of artificial 35 textile materials of improved properties, which comprises stretching at temperatures of at least 90° C. during their travel from one point to another artificial filaments, yarns and like textile materials having a basis of cellulose acetate, containing a proportion of at least 40% on the weight of the cellulose acetate of a plasticizer for the cellulose acetate which is compatible therewith 40 in a proportion of at least 50% and containing substantially no volatile softening agent.

6. Process for the manufacture of artificial 45 textile materials of improved properties, which comprises stretching to at least 200% of their original length and during their travel from one point to another at temperatures of at least 90° C. artificial filaments, yarns and like textile materials having a basis of cellulose acetate, containing a proportion of at least 60% on the weight 50 of the cellulose acetate of a plasticizer for the cellulose acetate which is compatible therewith in a proportion of at least 100% and containing substantially no volatile softening agent.

7. Process for the manufacture of artificial 55 textile materials of improved properties, which comprises forming artificial filaments, yarns and like textile materials having a basis of cellulose acetate and containing at least 60% of their weight of a plasticizer for the cellulose acetate which is compatible therewith in a proportion of at least 100% by an evaporative process from a spinning solution containing the cellulose acetate and the plasticizer, and then stretching said 60 materials to at least 200% of their original length during their travel from one point to another at a temperature of at least 90° C. while they are substantially free from volatile softening agent. 65